

## UNITED STATES PATENT OFFICE

2,229,137

## PRODUCTION OF COLOR PHOTOGRAPHS

Wilhelm Schneider, Dessau, Germany, assignor,  
by mesne assignments, to General Aniline &  
Film Corporation, New York, N. Y., a corpora-  
tion of Delaware

No Drawing. Application June 17, 1937, Serial  
No. 148,731. In Germany June 26, 1936

3 Claims. (CL. 95—2)

The present invention relates to color photographs.

One of its objects is to provide an improved process of producing multi-color photographs.

5 Further objects will be seen from the detailed specification following hereafter.

It has been proposed to prepare by the reversal process color pictures from a multi-layer material, individual layers of which contain dyestuff formers, and to apply the chromogenic development only for the second development.

When this process is applied in practice, for example for narrow films, it is necessary either that the existing developing machines should be 15 so constructed that they are applicable both for black and white reversal pictures in the usual manner and for chromogenic second development, or to provide separate developing machines for exposures to be chromogenically developed. 20 The latter would considerably increase the cost of an installation.

This invention relates to a novel chromogenic developing process which differs from those that are known as follows:

25 The material is developed after the exposure in the existing developing machines in any known manner to produce a black and white reversal positive. On inspection the picture obtained cannot be distinguished from an ordinary 30 reversal positive. In fact, however, this positive consists of component positives in the layers which constitute the multi-layer material. The layers contain the still unchanged dyestuff components as described for instance in U. S. patent 35 applications Ser. No. 72,718 filed April 4, 1936; Ser. No. 90,726 filed July 15, 1936; Ser. No. 94,340 filed August 5, 1936; and Ser. No. 126,842 filed February 20, 1937.

In a simple developing apparatus this material is now subjected in daylight to re-sensitizing, and then the silver component pictures changed into exposed silver salts are developed to color pictures containing silver, from which pictures the silver may be removed in known manner, for instance by the Farmer's reducer.

45 This process of developing requires merely the installation of a simple additional apparatus requiring but little manipulation. The finishing of the black and white positive affords an opportunity for examining the picture and noting any corrections which may be necessary, these being made before the final color development.

The following example serves to illustrate the invention:

50 A photographic multi-layer material compris-

ing a support, a silver halide gelatin emulsion layer sensitized to red and containing the sodium salt of 1-N-stearoyl-4-N-(1'-hydroxy-2-naphthoyl)-phenylenediaminesulfonic acid as a dyestuff component, a second emulsion layer sensitized to green and containing 1-(5'-sulfo-3'-stearoylaminophenyl)-pyrazolone sodium as a dyestuff component and a not specially sensitized third emulsion layer containing m-stearoyl-amino-benzoylacetanilide-p'-carboxylic acid as a 10 dyestuff component is exposed and developed in the following working steps:

1. First development with Amidol

The multi-layer material is treated for 15 minutes in an Amidol developer consisting of 1000 cc. of water, 5 grams of Amidol, 50 grams of sodium sulfite sicc. and 1 gram of potassium bromide and then washed for 10 minutes.

2. First bleaching with chromic acid

The material is treated for 8-9 minutes in a composition of 1000 cc. of water, 5 grams of chromic anhydride and 30 grams of sodium sulfite sicc. or in a composition of 1000 cc. of water, 4 grams of potassium bichromate and 25 cc. of sulfuric acid of 10 per cent strength and then washed for 10 minutes. After clarifying for 2 minutes in a sodium sulfite solution of 3 per cent strength the material is washed for 5 minutes.

3. Re-exposure

4. Second development with Amidol

After developing for 10 minutes in a composition of 1000 cc. of water, 5 grams of Amidol, 50 grams of sodium sulfite sicc. and 1 gram of potassium bromide or for 5 minutes in an Agfa I negative developer the material is washed for 10 minutes.

5. Second bleaching with chromic acid

The material is treated for 3 minutes in a composition of 1000 cc. of water, 5 grams of chromic anhydride and 50 grams of sodium chloride or in a solution of 1000 cc. of water, 4 grams of potassium bichromate, 25 cc. of hydrochloric acid of 10 per cent strength and 20 grams of sodium chloride and then washed for 10 minutes.

6. Second re-exposure

7. Color development

After a treatment for 10 minutes in a bath containing 1000 cc. of water, 0.5 gram of sodium sulfite sicc., 2.5 grams of p-diethyl-amino-an-

line, 2.5 grams of potassium bromide and 30 grams of sodium carbonate the material is washed for 25 minutes.

5 8. *Bleaching with potassium ferricyanide*

The material is treated for 6 minutes in a solution of 1000 cc. of water, 50 grams of potassium ferricyanide and 50 grams of sodium chloride.

10 9. *Fixing*

The bath is made by dissolving 300 grams of sodium thiosulfate in 1000 cc. of water.

The temperature of the above cited baths is 18° C.

15 15. The latent image necessary for the color development is produced by exposure or in a chemical manner. There is no need to effect the various working steps immediately following each other. It is for instance possible to interrupt the development after the third step and to effect the bleaching and subsequent color development only after a considerable interval. In this manner it is possible to develop the latent image even in cases where only the usual developing agents 20 are at hand, thereby keeping it from being deleteriously affected.

25 What I claim is:

30 1. A process of producing multi-color photographs which comprises producing a multi-layer photographic material having incorporated in the several silver halide emulsion layers dyestuff components capable of forming dyestuffs with a developer adapted for color development, said dyestuff component although soluble in aqueous liquids being per se incapable of diffusing with respect to the binding agent of the emulsion layer, forming positive silver component images in said layers by a reversal process with processing solutions which are incapable of forming dyestuffs 35 with said dyestuff components, bleaching said silver images to silver salt images, rendering said silver salt images developable, transforming said images into silver and color component images in a developer capable of forming dyestuffs with said dyestuff components, and removing the developed silver from said photographic material.

2. A process of producing multi-color photographs, which comprises producing a multi-layer film having incorporated in the several silver halide emulsion layers dyestuff components capable of forming dyestuffs with a developer adapted for color development, said dyestuff components being fast to diffusion with respect to the binding agent of the emulsion layer, forming latent images, developing said images in a developer not capable of forming dyestuffs with 10 said dyestuff components, dissolving the silver from the negative by treatment in a bleaching bath, forming latent images in the remaining silver halide, developing said images in a developer corresponding to the first development step, 15 forming silver halide images by treatment in a bleaching bath, forming latent images, transforming said images into silver and color images in a developer capable of forming dyestuffs with 20 said dyestuff components, and removing the developed silver from said film.

3. A process of producing multi-color photographs, which comprises producing a multi-layer film having incorporated in the several silver halide emulsion layers dyestuff components capable of forming dyestuffs with a developer adapted for color development, said dyestuff components being fast to diffusion with respect to the binding agent of the emulsion layer, forming latent images, developing said images in a developer not capable of forming dyestuffs with said dyestuff components, dissolving the silver from the negative by treatment in a bleaching bath, forming latent images in the remaining silver halide, developing said images in a developer corresponding to the first development step, 30 forming silver halide images by treatment in a bleaching bath, forming latent images, transforming said images into silver and color images in a developer capable of forming dyestuffs with said dyestuff components, removing the developed silver from said film, and fixing the produced colored positive.

WILHELM SCHNEIDER. 45